

# UNITED STATES PATENT OFFICE.

JOHN F. THOMPSON, OF BROOKLYN, AND EDWARD E. SEELYE, OF TOMPKINSVILLE, NEW YORK, ASSIGNEES, BY MESNE ASSIGNMENTS, TO THE INTERNATIONAL NICKEL COMPANY, A CORPORATION OF NEW JERSEY.

## PROCESS OF PREVENTING OXIDATION OF METALS DURING ANNEALING.

1,085,768.

Specification of Letters Patent.

Patented Feb. 3, 1914.

No Drawing.

Application filed March 8, 1912. Serial No. 682,538.

*To all whom it may concern:*

Be it known that we, JOHN F. THOMPSON, a citizen of the United States, residing in Brooklyn, Kings county, New York, and EDWARD E. SEELYE, a citizen of the United States, residing at Tompkinsville, Richmond county, New York, have invented an Improved Process of Preventing Oxidation of Metals During Annealing, of which the following is a specification.

Our invention relates to the annealing of metals and is especially directed to the prevention or elimination of oxidation on the surface of metals during the annealing operation. We have discovered that when a fusible halogen salt of an alkaline or an alkaline-earth metal is mixed with a base and spread on the article to be annealed, that during the annealing operation the article will not oxidize, and, moreover, not only is oxidation prevented, but such halogen salt will act as a solvent to remove any oxid on the surface of the metal when it is heated for annealing.

The following is a typical way of carrying out our method: To boiling water in a suitable receptacle, we add calcium chlorid, and the calcium chlorid is thereby dissolved in the water and forms a saturated solution of calcium chlorid. We then emulsify the mixture by adding ground fluorspar (calcium fluorid) and the result is a mixture in the form of a thin paste. To this, if desired, we may add more water for the purpose of thinning the mixture. We then apply the paste to the article to be annealed by either dipping the article into the paste or by applying the paste to the article with a brush. When the article is heated, its surfaces, instead of oxidizing, are kept free from oxidation, and after annealing the paste can be washed, rubbed, or brushed off, and the surfaces of the article are found in substantially the same condition in which they were before annealing. If, however, the article was somewhat oxidized before annealing, such oxid will be found to have

been removed during the annealing operation, the mixture acting as a solvent therefor during the heating operation.

In the typical method we usually employ two parts of fluorspar to one part of calcium chlorid, the calcium chlorid being the active agent and the fluorspar being the base which retains the calcium chlorid on the surface of the article when the calcium chlorid fluxes from the heat during the annealing process. The base employed must act as a vehicle to retain the active agent on the surfaces of the articles during the annealing temperature, since if the mixture is not retained on the surfaces of the articles in a uniform manner, oxidization will ensue. The water is added to aid in spreading the mixture on the article to be annealed.

The proportions of the base and of the fusible halogen salt of an alkaline-earth metal may be varied within certain limits in the practice of our invention, and any material may be used instead of the calcium fluorid which will act as a suitable vehicle for the active agent.

Where we mention in the claims an alkaline metal, it is to be understood that we designate an alkaline or an alkaline earth metal, which have properties that are the same for our purpose.

What we claim is:

1. The process of annealing metallic articles, which consists in applying to the surfaces of articles to be annealed, a mixture composed of fluorspar and calcium chlorid, and then heating the articles for annealing thereby preventing oxidation of the articles during annealing.

2. The process of annealing metallic articles, which consists in applying to the surfaces to be annealed, a mixture composed of two parts calcium fluorid and one part calcium chlorid, and then heating the articles for annealing thereby preventing oxidation of the articles during annealing.

3. The process of annealing metallic articles, which consists in applying to the sur-

50

60

65

70

75

80

85

90

faces to be annealed, an emulsion composed of calcium fluorid, calcium chlorid and water, and then heating the articles for annealing thereby preventing oxidation of the 5 articles during annealing.

4. The process of preventing oxidization during annealing, which consists in applying to the surfaces of the articles to be an-

nealed a mixture comprised of calcium fluorid and a fusible halogen salt of an 10 alkaline metal.

JOHN F. THOMPSON.  
EDWARD E. SEELYE.

Witnesses:

LUCIUS R. COSTIZA,  
LUKE E. GRAHAM.